

## 1

2,947,700

## INHIBITED CHLORITE BATHS AND METHOD

Wilhelm Waibel, Frankfurt am Main, Germany, assignor to Farbwerke Hoechst Aktiengesellschaft vormals Meister Lucius & Bruning, Frankfurt am Main Hochst, Germany, a company of Germany

No Drawing. Filed Oct. 2, 1956, Ser. No. 613,364

Claims priority, application Germany Dec. 15, 1953

6 Claims. (Cl. 252—102)

This application is a continuation-in-part application of my co-pending application Ser. No. 474,607, filed December 10, 1954, now abandoned, on: "Compositions Suitable for Diminishing the Formation of Chlorine Dioxide in Acid Chlorite Baths and a Method of Such Diminishing."

In working with aqueous acid solutions of chlorites a certain amount of chlorine dioxide always escapes from the baths and this constitutes a great danger and annoyance to the operatives. The escape of chlorine dioxide from acid chlorite baths gives rise to considerable technical difficulties and attempts have been made to overcome this inconvenience by using suction and absorption devices. These expedients are highly expensive and the loss of valuable material is inevitable.

In order to diminish the amount of chlorine dioxide evolved from the chlorite baths, it has been proposed to add various substances, for example, peroxides, and preferably hydrogen peroxide, to the acid chlorite baths. This expedient involves an additional consumption of the costly bleaching agent. It is also known to add fluorine compounds, and preferably acid fluorides, such as ammonium difluoride, to the acid chlorite baths, in order to suppress the evolution of chlorine dioxide. Apart from the fact that these fluorine compounds do not constitute an adequate remedy, they have the further disadvantage that they attack refined steel as well as ceramic material which is relatively resistant to the acid chlorine solutions. It is also known to inhibit corrosion when working with aqueous solutions of chlorites or chlorine dioxide in apparatus of refined steel, by adding nitrates, for example, ammonium nitrate to the baths.

Now I have found that the formation of chlorine dioxide in acid chlorite baths can be diminished by adding to the baths ammonium chloride, ammonium sulphate, ammonium chlorate or an ammonium salt of an aliphatic carboxylic acid of low molecular weight and a sulphonate acid and/or carboxylic acid containing an aliphatic radical of high molecular weight interrupted by a carboxylic acid amide or carboxylic acid ester group or a salt of such acid of high molecular weight.

The proportions in which the above mentioned ammonium salts are to be added per litre of liquor may vary within wide limits. An addition of about 0.5 to about 2 grams per litre of liquor generally suffices. For reasons of economy a proportion within the range of about 0.6 to 1 gram may be used, although proportions smaller or larger than those mentioned above, for example, 0.3 or 5.0 grams, may be added.

The proportions of the sulphonate acid and/or carboxylic acid, or the salts thereof, containing an aliphatic radical of high molecular weight interrupted by a carboxylic acid amide or carboxylic acid ester group may also vary within wide limits. It is possible to add quantities equal to, inferior to or larger than the quantity of ammonium salt used. In many cases it is sufficient to use about one fourth of the amount of ammonium salt. Normally, quantities will be used amounting to one fourth up to the

## 2

equal amount by weight of ammonium salt used. In special cases it might, however, be advisable to use more than the equal quantity by weight, for instance double or three times up to 10 times its amount. In general, however, the effect is not increased by using higher quantities of the surface-active substances claimed. Sometimes, it is also sufficient to add inferior quantities; in some cases the amount can be reduced to about  $\frac{1}{25}$  of the quantity of ammonia salt used.

10 In addition to the substances mentioned above, there may also be added to the chlorite baths the additions customarily used for adjusting the pH-value, for example, hydrochloric acid, formic acid, acetic acid, oxalic acid, phosphoric acid, nitric acid, bisulphates such as sodium bisulfate, acid ortho-phosphates, pyrophosphates, acid polymeric phosphates or mixtures of these acid compounds, and the like.

15 In order to avoid corrosion when working in apparatus of refined steel, it is of advantage to add acids of the oxides of nitrogen or salts thereof.

20 As sulfonic and/or carboxylic acids of high molecular weight there enter into consideration reaction products as are obtained for instance by causing fatty acids of high molecular weight i.e. such containing more than 8 carbon atoms on amino-sulphonic or amino-carboxylic acids of low molecular weight or on protein decomposition products. Furthermore, there are to be mentioned the condensation products of the salts from the above-mentioned fatty acids and halogen-sulphonic acids or halogen-car-

25 boxylic acids. The products can also be obtained by causing fatty acid derivatives to act upon aliphatic hydroxy-carboxylic acids of low molecular weight. Such compounds are disclosed, for instance, by Schwartz-Perry "Surface Active Agents," 1949, pages 34-39, 94-97 and

30 102-103. There are mentioned for example the reaction products of fatty acids, particularly in the form of their chlorides, containing more than 8 carbon atoms, especially those containing 12-18 carbon atoms, as, for instance, lauric acid, myristic acid, palmitic acid, stearic acid, or oleic acid with amino acetic acid, taurine, methyltaurine, methyl-amino acetic acid, hydroxymethane- or hydroxyethane-sulfonic acid, tartaric acid and the like, for instance lauryl-methyl-tauride, oleyl-methyl-tauride, myristyl- and palmityl-tauride, stearyl tauride, stearoxy-methane and stearoxy-ethane-sulphonic acid, laurylsarcoside, stearylsarcoside, stearate of tartaric acid obtained by reaction of stearic acid chloride in dry pyridine on tartaric acid, etc.

35 The invention also includes a solid composition suitable for diminishing the formation of chlorine dioxide in acid chlorite baths, which comprises ammonium chloride, ammonium sulphate, ammonium chlorate or an ammonium salt of an aliphatic carboxylic acid of low molecular weight and a sulphonate and/or carboxylic acid containing an aliphatic radical of high molecular weight interrupted by a carboxylic acid amide or carboxylic ester group or a salt of such acid of high molecular weight. Such a composition is stable, and provides a mixture of the ingredients in the appropriate relative proportions, so that, when required for use, there can be prepared therewith an aqueous solution containing a suitable quantity of the composition.

40 In order to inhibit corrosion when working with chlorite baths in apparatus made of refined steel, a salt of an acid of an oxide of nitrogen, advantageously sodium nitrate, may also be incorporated in the above composition. Such compositions are very stable.

45 As an alternative to solid compositions, the invention also provides concentrated aqueous solutions of the ingredients mentioned above. Such concentrated solutions 50 are also stable. For use they need only be diluted with an appropriate quantity of water.

The solid compositions may be prepared by intimately mixing the ingredients together, the separate ingredients advantageously being of the same particle size. Alternatively, the solid compositions may be prepared by the evaporation or spray drying of a solution of the ingredients.

Other additions of the kind customary in chlorite baths may be incorporated with the solid compositions or concentrated solutions or, depending on the nature of the addition, with the solutions to be used. As compared with the use of ammonium nitrate together with a surface-active substance of the kind used in the present invention, the use of the ammonium salts of this invention together with the said surface-active substances results in a substantially improved decrease in the formation of chlorine dioxide.

This is evident, for example, from the decrease in the content of chlorite of a solution containing, per litre, 2.5 grams of sodium chlorite and 0.3 gram of a condensation product of a fatty acid with protein degradation products at a temperature of 60° C. and a pH value of 3.3, which is brought about by the addition to separate portions of the solution of various quantities of ammonium nitrate or certain of the ammonium salts used in this invention. In the following table are given the quantities of ammonium salts added and the decrease in the chlorite content in the course of one hour. The extreme right-hand column indicates the percentage by which the decrease in the chlorite content is reduced by using, instead of ammonium nitrate, an equal quantity of an ammonium salt in accordance with the present invention:

| Quantity of ammonium nitrate in g./l. | Decrease in chlorite content in g./l. | Ammonium salt in same quantity instead of ammonium nitrate | Decrease in chlorite content in g./l. | Percentage reduction in decrease in chlorite content as compared with the use of ammonium nitrate |
|---------------------------------------|---------------------------------------|------------------------------------------------------------|---------------------------------------|---------------------------------------------------------------------------------------------------|
| 0.8                                   | 0.19                                  | ammonium chloride                                          | 0.09                                  | 53                                                                                                |
| 0.6                                   | 0.18                                  | ammonium sulphate                                          | 0.12                                  | 33                                                                                                |
| 0.75                                  | 0.18                                  | ammonium acetate                                           | 0.10                                  | 45                                                                                                |
| 1.0                                   | 0.18                                  | ammonium chlorate                                          | 0.08                                  | 56                                                                                                |

Furthermore, the solutions containing ammonium nitrate exhibit a yellow-olive coloration after one hour, whereas those containing ammonium chloride, ammonium sulphate, ammonium acetate or ammonium chlorate are still nearly colorless after that time.

The advantages are similar with regard to the known use of acid fluorides, for example ammonium bifluoride. Thus, a solution containing, per litre, 1 gram of sodium chlorite and 0.5 gram of ammonium bifluoride, and having a temperature of 60° C. and a pH value of 3.5 undergoes a decrease in chlorite content of 9 percent after one hour and exhibits an olive coloration due to free chlorine dioxide. On the other hand, a sodium chlorite solution of the same concentration which contains, instead of ammonium bifluoride, 0.5 gram of ammonium sulphate and 0.3 gram of oleyl methyl taurine undergoes under the same conditions a decrease in chlorite content of only 3.8 percent and furthermore remains colourless as hardly any free chlorine dioxide is split off.

The following examples serve to illustrate the invention but they are not intended to limit it thereto:

#### Example 1

A fabric of staple fibers of viscose was treated at 70° C. at a goods-to-liquor ratio of 1:20 with a solution con-

taining, per liter, 1 gram of sodium chlorite, 0.35 gram of oleyl-sarcoside and 0.6 gram of ammonium chloride whose pH value was adjusted to 3.4 by adding hydrochloric acid. The material thus bleached had a whiteness of 80.6 percent. The consumption of sodium chlorite amounted to 0.23 percent.

By the same procedure, but using 0.6 gram per liter of ammonium nitrate instead of ammonium chloride, 0.32 percent of sodium chlorite was consumed, i.e. about 39 percent more than with the use of ammonium chloride, and without a purer white being obtained.

The above-mentioned quantities of surface-active agents and ammonium chloride and also the relative proportions thereof may vary within wide limits. By increasing the quantities of the additions the rate of bleaching can be substantially reduced as required, and it is possible to work without any production of odour and also a substantial saving of chlorite can thus be achieved.

#### Example 2

A fabric of staple fibers of viscose was treated at 70° C. at goods-to-liquor ratio of 1:20 with a solution containing, per liter, 1 gram of sodium chlorite, 0.35 gram of lauryl-sarcoside and 0.75 gram of ammonium chlorate whose pH value was adjusted to 3.4 by adding acetic acid. The material thus bleached had a whiteness of 80.6 percent. The consumption of sodium chlorite was 0.24 percent.

By the same procedure, but using 0.75 gram per liter of ammonium nitrate instead of ammonium chlorate, 0.33 percent of sodium chlorite was consumed, i.e. almost 38 percent more than with the use of ammonium chlorate, and without a purer white being obtained.

The above-mentioned quantities of surface-active agents and ammonium chlorate and also the relative proportions thereof may vary within wide limits. By increasing the quantities of the additions the rate of bleaching can be substantially reduced as required, and it is possible to work without any production of odour and also a substantial saving of chlorite can thus be achieved.

#### Example 3

A fabric of staple fibers of viscose was treated at 70° C. at a goods-to-liquor ratio of 1:20 with a solution containing, per liter, 1 gram of sodium chlorite, 0.35 gram of the sodium salt of the esterification product from oleic acid and isethionic acid and 0.7 gram of ammonium sulphate and having a pH value of 3.4 adjusted by the addition of formic acid. The material thus bleached had a whiteness of 80.7 percent. The consumption of sodium chlorite was 0.27 percent.

By the same procedure, but using 0.7 gram per liter of ammonium nitrate instead of ammonium sulphate, 0.33 percent of sodium chlorite was consumed, i.e. about 22 percent more than with the use of ammonium sulphate, and without a purer white being obtained.

The above-mentioned quantities of surface-active agents and ammonium sulphate and also the relative proportions thereof may vary within wide limits. By increasing the quantities of the additions the rate of bleaching can be substantially reduced as required, and it is possible to work without any production of odour and also a substantial saving of chlorite can thus be achieved.

#### Example 4

A fabric blended from staple fibers of viscose and cotton was treated at 70° C. at a goods-to-liquor ratio of 1:20 with a solution containing, per liter, 1 gram of sodium chlorite, 0.35 gram of the sarcoside of coconut oil fatty acids and 0.6 gram of ammonium acetate and having a pH value of 3.4 adjusted by addition of phosphoric acid. The material thus bleached had a whiteness of 80.6 percent. The consumption of sodium chlorite

was 0.26 percent. By the same procedure, but using 0.6 gram per liter of ammonium nitrate, instead of ammonium acetate, 0.32 percent of sodium chlorite was consumed, i.e. about 27 percent more than with the use of ammonium acetate, and without a purer white being obtained.

The above-mentioned quantities of surface-active agents and ammonium acetate and also the relative proportions thereof may vary within wide limits. By increasing the quantities of the additions the rate of bleaching can be substantially reduced as required, and it is possible to work without any production of odour and also a substantial saving of chlorite can thus be achieved.

*Example 5*

A fabric of staple fibers of viscose was treated for 40 minutes at 75° C. at a goods-to-liquor ratio of 1:20 with a solution containing, per liter, 1 gram of sodium chlorite, 2 grams of ammonium nitrate, 5 grams of ammonium sulphate and 0.2 gram of oleyl-methyl-tauride and having a pH value of 3.5, adjusted by addition of mono-sodium phosphate and then rinsed. The material thus bleached had a whiteness of 79.8 percent. The consumption of sodium chlorite was not more than 0.18 percent. No liberation of chlorine dioxide occurred. Instead of the aforesaid quantity of ammonium sulphate, the same quantity of ammonium chloride or ammonium acetate may be used.

The above-mentioned quantities of surface-active agents and ammonium sulphate and also the relative proportions thereof may vary within wide limits. By increasing the quantities of the additions the rate of bleaching can be substantially reduced as required, and it is possible to work without any production of odour and also a substantial saving of chlorite can thus be achieved.

*Example 6*

A fabric of staple fibers of viscose was treated for 40 minutes at 75° C., at a goods-to-liquor ratio of 1:20 with a solution containing, per liter, 1 gram of sodium chlorite, 0.3 gram of ammonium chloride and 3 grams of lauryl-methyltauride and having a pH value of 3.5 adjusted by addition of formic acid, and then rinsed.

The material thus bleached had a whiteness of 80.2 percent. The consumption of sodium chloride did not exceed 0.21 percent. No chlorine dioxide escaped during the bleaching process. Instead of the aforesaid quantity of ammonium chloride, the same quantity of ammonium sulphate, ammonium chlorate or ammonium acetate may be used.

*Example 7*

Knit goods of staple fibers of cellulose acetate were treated for 20 minutes at 70° C., at a goods-to-liquor ratio of 1:25, with a solution containing per liter 1.5 grams of calcium chlorite, 0.4 gram of ammonium chloride and 2 grams of lauric acid methyl tauride, as well as 1 gram of stearic acid sarcoside. The pH value of the bleaching bath was adjusted to 3.0 by means of a mixture consisting of sodium acetate and hydrochloric acid in a proportion of 1:1.

During the bleaching process no escaping of chlorine dioxide was observed. An excellent bleaching result was obtained. The bleached knit goods were of agreeable handle.

*Example 8*

Yellowed yarn of polyamide fibers consisting of hexamethylene diamine and adipic acid were treated for 1 hour at 85° C. in a bleaching bath containing per liter 1 gram of sodium chlorite, 2 grams of ammonium acetate and 1 gram of myristyloxy-ethansulfonic acid ammonium and showing a pH value of 4.5 adjusted by means of oxalic acid. Escaping chlorine dioxide was not observed. The bleaching effect was good.

*Example 9*

A fabric of polyester fibers from polyethylene glycol terephthalate was treated in a goods-to-liquor ratio of 1:30 with a solution containing per liter 2 grams of sodium chlorite, 3 grams of ammonium phosphate, 2 grams of a condensation product of fatty acids of tallow and hydrolyzed protein and 1 gram of acid sodium hexamethaphosphate and adjusted to a pH value of 2.5 by the addition of nitric acid. The bleaching process was carried out at 80° C. within 20 minutes. Then the fabric was rinsed and dried. An annoyance by escaping chlorine dioxide was not observed when realizing the process in this way. A very satisfactory bleaching effect was obtained.

15 I claim:

1. A method of diminishing the formation of chlorine dioxide in acid sodium chlorite baths used for bleaching textile materials and having a pH of about 2.5 to 4.5, comprising adding to said baths an ammonium salt selected from the group consisting of ammonium chloride, ammonium sulphate, ammonium chlorate and ammonium acetate in a concentration of about 0.3 to 5 grams per liter and further adding a compound selected from the group consisting of sulfonic acids and carboxylic acids containing an aliphatic radical having eight to eighteen carbon atoms which is interrupted by a carboxylic amide group and of sulphonated acids and carboxylic acids containing an aliphatic radical having eight to eighteen carbon atoms which is interrupted by a carboxylic ester group and the salts thereof.

2. A method of diminishing the formation of chlorine dioxide in acid sodium chlorite baths used for bleaching textile materials and having a pH of about 2.5 to 4.5, comprising adding to said baths ammonium chloride in a concentration of about 0.3 to 5 grams per liter and further adding the sodium salt of a sulfonic acid containing an aliphatic radical having eight to eighteen carbon atoms which is interrupted by a carboxylic amide group.

3. A method of diminishing the formation of chlorine dioxide in acid sodium chlorite baths used for bleaching textile materials and having a pH of about 2.5 to 4.5, comprising adding to said baths ammonium sulphate in a concentration of about 0.3 to 5 grams per liter and further adding the sodium salt of a sulfonic acid containing an aliphatic radical having eight to eighteen carbon atoms which is interrupted by a carboxylic amide group.

4. A method of diminishing the formation of chlorine dioxide in acid sodium chlorite baths used for bleaching textile materials and having a pH of about 2.5 to 4.5, comprising adding to said baths ammonium chlorate in a concentration of about 0.3 to 5 grams per liter and further adding the sodium salt of a sulfonic acid containing an aliphatic radical having eight to eighteen carbon atoms which is interrupted by a carboxylic amide group.

5. A method of diminishing the formation of chlorine dioxide in acid sodium chlorite baths used for bleaching textile materials and having a pH of about 2.5 to 4.5, comprising adding to said baths ammonium acetate in a concentration of about 0.3 to 5 grams per liter and further adding the sodium salt of a sulfonic acid containing an aliphatic radical having eight to eighteen carbon atoms which is interrupted by a carboxylic amide group.

6. In the bleaching of a textile material by immersion in an aqueous solution of acid sodium chlorite having a pH of about 2.5 to 4.5, the improvement which comprises carrying out the bleaching operation in the presence of an ammonium salt of the group consisting of ammonium chloride, ammonium sulfate, ammonium chlorate and ammonium acetate in a concentration of about 0.3 to 5 grams per litre and a compound of the group consisting of sulfonic acids and the carboxylic acids containing an aliphatic radical having eight to eighteen carbon atoms which is interrupted by a carboxylic amide

group and of sulfonic acids and carboxylic acids containing an aliphatic radical having eight to eighteen carbon atoms which is interrupted by a carboxylic ester group and the salts thereof.

References Cited in the file of this patent

UNITED STATES PATENTS

2,353,823 Hampel July 18, 1944  
2,415,657 Riggs et al. Feb. 11, 1947

5 2,526,839  
2,607,738  
2,691,637  
2,694,059  
2,711,363

2,739,032  
2,747,734

461,328

Aston Oct. 24, 1950  
Hardy Aug. 19, 1952  
Waibel Oct. 12, 1954  
Lamborn et al. Nov. 9, 1954  
Waibel June 21, 1955  
Wilson Mar. 20, 1956  
Reese et al. May 29, 1956

FOREIGN PATENTS

Great Britain Feb. 15, 1937